# EUROPEAN PATENT SPECIFICATION

(11) **EP 0 045 815 B1**
(45) Date of publication and mention of the grant of the patent: **11.07.1984**
(21) Application number: 80104708.5
(22) Date of filing: 11.08.1980
(51) Int. Cl.: C22C 38/60, C21C 7/00, C21D 7/13

(54) **Semi-finished steel article and method for producing same**
Vorgearbeiteter Stahlartikel und Verfahren zu seiner Herstellung
Produit semi-fini en acier et procédé pour sa fabrication

(43) Date of publication of application: 17.02.1982
(73) Proprietor: INLAND STEEL COMPANY, Chicago, IL 60603 (US)
(72) Inventor: Bhattacharya, Debanshu, Matteson Illinois (US); Holowaty, Michael O., Crown Point Indiana (US); Quinto, Dennis T., St. John Indiana (US)
(74) Representative: Leach, John Nigel

## Description

The present invention relates generally to elongated semi-finished, free machining steel shapes and more particularly to such shapes which are free of surface cracking and to methods for producing such shapes.

A semi-finished steel shape is a bloom or a billet, the latter having a smaller cross-section than the former, produced from an ingot or a continuously cast strand having a cross-section similar to that of a bloom or billet and which has been subjected to a hot deforming operation such as roll straightening.

The machinability of steel is increased by adding alloying ingredients such as sulphur, lead, tellurium and bismuth.

In one type of manufacturing operation for producing a semi-finished steel shape having a free machining composition, molten steel, containing at least some of the machinability increasing ingredients described above, is poured into an ingot mould where the steel is cast into an elongated solid shape. After cooling, the ingot is reheated and subjected to a hot rolling operation which rolls the ingot into a bloom, and the bloom is then reheated and subjected to a further hot rolling operation to form the bloom into a billet. The billet is subsequently rolled into a bar, which is a finished steel shape.

In another form of manufacturing operation, for producing a semi-finished steel shape having a free machining composition, the steel is continuously cast as strands having the cross-section of a billet, the strand is subjected to a roll bending operation or a roll straightening operation while the steel is at a hot deforming temperature, and, after the roll straightening operation, the strand is cut into billet lengths (which comprise semi-finished steel shapes).

The hot rolling of the ingot into a bloom and the hot rolling of the bloom into a billet are generally performed at a hot rolling temperature in the range 920⁰⁻1150⁰C (1700°-2100°F). The roll straightening of a continuously cast strand is generally performed at a temperature in the range 920⁰⁻1100°C (17000-20000 F). The hot rolling of the ingot into a bloom, the hot rolling of the bloom into a billet, and the roll straightening of the continuously cast strand are all hot deforming operations, and the temperature ranges described above are the typical, normal temperature ranges used for these hot deforming operations.

When tellurium is present in a free machining steel, all the tellurium is in inclusion form, principally as lead telluride (PbTe) when lead is also present. Some of the tellurium may also be present as manganese telluride (MnTe).

In steels containing lead and tellurium, and undesirable phenomenon occurs at the temperature range normally utilised for hot deforming. This phenomenon, known as surface cracking or surface checking or surface tearing, is manifest by a large number of small cracks or checks at the surface of the semi-finished steel shape, particularly along the corners. Severe surface checking renders a steel shape commercially unacceptable.

Surface cracking has been recognised in the prior art and attempts to combat this phenomenon have -also been described in the prior art. More specifically, attempts to combat surface cracking include reheating the unfinished steel shape without flame impingement on the surface of the unfinished shape (U.S. Patent No. 3,287,954 Scrader et al), reducing the moisture content in the atmosphere of the reheating furnace (U.S. Patent No. 3,365,922 Conces et al), removing the surface and first sub-layer of the unfinished steel shape, e.g. by scarfing, after reheating (U.S. Patent No. 3,382,700 Heitmann et al) and providing a blanket of non-oxidizing gas around the steel shapes as they undergo reheating (U.S. Patent No. 3,710,608 Hentz et al).

Typical examples of steel containing both lead and tellurium are disclosed in Holowaty U.S. Patent No. 3,152,889.

In accordance with one aspect of the present invention we provide a method for producing a free-machining, elongated, semi-finished, tellurium containing steel shape devoid of surface cracking, prior to any surface conditioning thereof, due to lead telluride, characterised in that said method comprises the steps of:
providing a bath of molten steel having a composition comprising, in wt. %:
casting said molten steel into an elongated solid shape;
said steel being provided with sufficient manganese and bismuth so that, in said solid shape, all of the tellurium is combined with said manganese and/or said bismuth as micro-inclusions of MnTe and/or Bi₂Te₃ (except that when lead is present some of the tellurium may be combined with lead as micro-inclusions of PbTe in amounts insufficient to produce substantial surface cracking during hot forming of said billet) and said bismuth is also present as micro-inclusions of elemental bismuth, there being substantially no FeTe present in said solid shape;
heating said elongated steel shape to a hot deforming temperature, without burning the steel shape;
and hot deforming said elongated shape while the latter is at a temperature above about 920°C (1700°F) and below 1150°C (2100°F).

In accordance with another aspect of the invention, we provide an as-deformed billet of free machining steel characterised in that said billet comprises:
a composition comprising, in wt. %:
all of said tellurium being combined with said manganese and/or said bismuth as micro inclusions of MnTe and/or Bi₂Te₃ (except that when lead is present some of the tellurium may be combined with lead as microinclusions of PbTe in amounts insufficient to produce substantial surface cracking during hot forming of said billet)
there being substantially no FeTe;
micro inclusions of elemental bismuth;
a billet surface substantially devoid of surface cracking and burning in the as-deformed condition; and iron oxide on the surface of said billet in said as-deformed condition.

The invention as claimed reduces or eliminates the above discussed problems of surface cracking.

In accordance with the present invention, it has been determined that, if the amount of lead telluride in the microstructure of the steel is substantially reduced, then the extent to which the steel undergoes surface cracking during hot deforming is also substantialiy reduced, if not entirely eliminated. However, to reduce the amount of lead telluride present requires a substantial reduction of either the lead content or the tellurium content or both, and this reduces the machinability of the steel which would be undesirable.

It has been determined that the susceptibility of the steel to surface cracking can be substantially minimised without reducing the machinability of the steel by completely replacing the lead with bismuth or by
(1) replacing a substantial part of the lead with bismuth; and
(2) substantially reducing the tellurium content of the steel.

These compositional changes have the net effect of eliminating or minimizing the formation of lead telluride.

In conventional free machining steels, lead is normally present in the range 0.25-0.35 wt. % and tellurium is normally present in the range 0.04-0.06 wt. %. In accordance with the present invention, the lead content is either eliminated entirely or, if not eliminated entirely, it is reduced from 0.25-0.35 wt. % to 0.15 wt. % maximum and the tellurium is reduced from 0.04-0.06 wt. % to 0.02 wt. % maximum. The reduction in machinability resulting from the lower lead and tellurium contents is offset by adding bismuth in the range of 0.10-0.40 wt. %.

In the absence of lead, instead of forming lead telluride, the tellurium is present either as bismuth telluride (Bi₂Te₃) or as manganese telluride (MnTe) which may be in the form of an eutectic with manganese sulphide (MnS). Where substantial amounts of manganese telluride are present in the microstructure of the steel (e.g. in the absence of lead), the hot deforming temperature should preferably be conductd within the range 920°-1035°C (1700⁰⁻1900⁰F). This is to offset the tendency of substantial amounts of manganese telluride to cause surface cracking during hot rolling at temperatures substantially exceeding 1035°C (1900°F), e.g. if the steel undergoes hot rolling at a temperature of about 1150°C (2100°F).

Other features and advantages are inherent in the subject matter claimed and disclosed or will become apparent to those skilled in the art from the following detailed description.

Embodiments of the invention will now be described in detail by way of example.

A free machining, elongated, semi-finished steel shape devoid of surface cracking in accordance with the present invention can be produced by a method utilising two different casting procedures, either ingot casting or continuous casting. No matter which casting procedure is utilised, the steel composition may be essentially the same, within the broad limits set forth below, in weight percent:

A machinability increasing amount of tellurium is generally about 0.02 wt. %, minimum. Up to 0.15 wt. % lead is optional.

A bath of molten steel having a composition within the range set forth above is then cast into an elongated solid shape such as an ingot. The amounts of manganese and bismuth, within the ranges set forth above, are sufficient so that, when the steel is in solid form and no lead is present, all of the tellurium is combined with the manganese and/or the bismuth as micro inclusions of manganese telluride and/or bismuth telluride and the bismuth is also present as micro inclusions of elemental bismuth, there being substantially no iron telluride (FeTe) present in the solid steel. Iron telluride has a detrimental effect from the standpoint of causing surface cracking during hot deforming.

After the steel has been cast into an ingot, and the ingot has cooled, the ingot is removed from the ingot mould, reheated (an operation known as soaking) and then subjected to a hot rolling operation at a hot rolling temperature in the range 920⁰⁻1150°C (1700⁰⁻2100°F) wherein the ingot is rolled into bloom. The resulting intermediate, hot deformed steel shape, i.e. the bloom, has a surface substantially devoid of surface cracking, prior to any surface conditioning of the bloom. The bloom is then reheated and hot rolled at a temperature in the range 920⁰⁻1150⁰C (1700⁰⁻2100⁰F) to produce a billet having a surface substantially free of surface cracking prior to any surface conditioning thereof, and there is no need to conduct a surface removal step between the bloom reheating step and the step of hot rolling the bloom into a billet.

Not only is the surface of the bloom or billet devoid of substantial surface cracking, but, also the surface is devoid of burning in the as-deformed condition, due to the fact that the steel shape is rolled at a temperature (1150°C maximum) (2100°F maximum), below that at which burning of the steel occurs.

In a manufacturing procedure wherein the billet is formed by a continuous casting operation, the steps comprise continuously casting molten steel (having a composition within the ranges set forth above) into a strand and then roll straightening the strand while the latter is at a temperature in the range 920°-1 100°C (17000-2000°F). The strand, which already has the cross-section of a billet, is then cut into the usual billet lengths.

The roll straightening step which the strand undergoes at the temperature range described above is tantamount to a hot deforming step, but the surface of the strand, and of the billets which are cut from the strand, are devoid of surface cracking and burning in the as-deformed condition.

A billet formed from either of the above described manufacturing procedures has an oxide on its surface in the billet's as-deformed condition. This is reflective of the fact that the billet has not undergone any surface conditioning. As used herein, the term "as-deformed condition" refers to the condition of the billet immediately after being hot rolled (or otherwise hot deformed) and before it undergoes any surface conditioning following the hot deforming step.

Surface conditioning is a procedure conventionally utilised to remove surface imperfections or portions from semi-finished steel articles after a hot deforming step and includes grinding, chipping, scarfing, planing and the like.

The combined lead plus bismuth content of the steel shape should be at least 0.25 wt. % to supply the desired machinability. Therefore, in that embodiment of the invention wherein lead is ; completely absent, the bismuth content should be at least 0.25 wt. %. In that embodiment of the invention wherein lead is present up to 0.15 wt. %, the bismuth may be less than 0.25 wt. % so long as the combined lead and bismuth content is 0.25 wt. % minimum.

In that embodiment of the invention in which some lead is added to the steel (up to 0.15 wt. % maximum), although there may be small amounts of lead tellurium micro inclusions in the steel, these amounts are insufficient to produce substantial surface cracking during the hot deforming step. This is because not only is the lead content limited to 0.15 wt. % maximum, in this embodiment, but also, the tellurium content is limited to 0.02 wt.% maximum.

The present invention may be applied to virtually all steel base compositions to which lead and tellurium have previously been added. Examples thereof are set forth in Holowaty U.S. Patent No. 3,152,889, and the disclosure therein is incorporated herein by reference. Examples of steel compositions in accordance with the present invention are contained in the table set forth below.

In all of the above steels A-D, the balance of the composition consists essentially of iron (plus the usual incidentals/impurities).

Generally speaking, the present invention may be applied to plan carbon steels having a base composition (i.e. a composition without lead, tellurium or bismuth) in the 1000 series, 1100 series or 1200 series of steels (AISI numbers) in which the lead, tellurium and bismuth contents are controlled as described above and which, in their solidified form, are subjected to hot deforming procedures (including hot deforming temperatures) as described above.

The present invention may also be applied to certain alloy steels to which lead and tellurium have heretofore been added, such as steels having compositions corresponding to AISI steels 4140, 4142 and 8620.

The foregoing detailed description has been given for clearness of understanding only, and no unnecessary limitations should be understood therefrom, as modifications will be obvious to those skilled in the art.

## Claims

1. A method for producing a free-machining, elongated, semi-finished, tellurium containing steel shape devoid of surface cracking, prior to any surface conditioning thereof, due to lead telluride, characterised in that said method comprises the steps of:
providing a bath of molten steel having a composition comprising, in wt. %:
casting said molten steel into an elongated solid shape;
said steel being provided with sufficient manganese and bismuth so that, in said solid shape, all of the tellurium is combined with said manganese and/or said bismuth as micro-inclusions of MnTe and/or Bi_{Z}Te₃ (except that when lead is present some of the tellurium may be combined with lead as micro-inclusions of PbTe in amounts insufficient to produce substantial surface cracking during hot forming of said billet) and said bismuth is also present as micro-inclusions of elemental bismuth, there being substantially no FeTe present in said solid shape;
heating said elongated steel shape to a hot deforming temperature, without burning the steel shape;
and hot deforming said elongated shape while the latter is at a temperature above about 920°C (1700°F) and below 1150°C (2100°F).

2. A method as recited in Claim 1 wherein said casting step comprises casting said molten steel into an ingot; and said hot deforming step comprises reheating said ingot and then hot rolling said reheated ingot into a bloom with said ingot at a hot rolling temperature above 920°C (1700°F) and below 1150°C (2100°F); there being no surface removal step between said reheating and said hot rolling step.

3. A method as recited in Claim 2 and further comprising reheating said bloom and then hot rolling said bloom at a temperature above 920°C (1700°F) and below 1150°C (2100°F) to produce a billet having a surface substantially free of surface cracking prior to any surface conditioning thereof; there being no surface removal step between said bloom reheating step and said last recited hot rolling step.

4. A method as recited in Claim 1 wherein. said casting step comprises continuously casting said molten steel into a strand; and said hot deforming step comprises roll straightening said strand while the latter is at a temperature above 920°C (1700°F) and below 1 100°C (2000°F).

5. A method as recited in any one of the preceding claims wherein said hot deforming step is performed at a temperature below 1035°C (1900°F).

6. A method as recited in any one of the preceding claims wherein said steel further contains up to 0.15 wt. % lead, and said tellurium content is 0.02 wt. % maximum said steel in said solid shape, having micro inclusions of PbTe in amounts insufficient to produce substantial surface cracking during said hot deforming step.

7. A method as recited in any one of the preceding claims wherein, when lead is present, the combined lead plus bismuth content, is at least 0.25 wt. %.

8. An as-deformed billet of free machining steel characterised in that said billet comprises:
a composition comprising, in wt. %:
all of said tellurium being combined with said manganese and/or said bismuth as micro inclusions of MnTe and/or Bi₂Te₃ (except that when lead is present some of the tellurium may be combined with lead as microinclusions of PbTe in amounts insufficient to produce substantial surface cracking during hot forming of said billet)
there being substantially no FeTe;
micro inclusions of elemental bismuth;
a billet surface substantially devoid of surface cracking and burning in the as-deformed condition; and iron oxide on the surface of said billet in said as-deformed condition.

9. A billet as recited in Claim 8 wherein said steel further contains up to 0.15 wt. % lead, said tellurium content is 0.02 wt. % maximum, said billet having microinclusions of PbTe in amounts insufficient to produce substantial surface cracking during hot forming of said billet.

10. A billet as recited in Claim 8 or Claim 9 wherein, when lead is present, the combined lead plus bismuth content is at least 0.25 wt. %.

11. A billet as recited in any one of Claims 8 to 10 wherein the amount of MnTe micro-inclusions is sufficient to cause surface cracking during hot-deforming at temperatures substantially exceeding 1 035°C (19000F).

## Revendications

1. Procédé pour fabriquer une forme en acier contenant du tellure, semi-finie, allongée, exempte d'usinage, dépourvue de fissuration de surface, préablement à tout traitement de surface de celle-cit, due au tellurure de plomb, caractérisé en ce que ledit procédé comprend les étapes consistant à:
fournir un bain d'acier fondu ayant une composition comprenant, en poids %:
couler ledit acier fondu sous une forme solide allongée;
lest acier étant pourvu de quantités suffisantes de manganèse et de bismuth pour que, dans ladite forme solide, tout le tellure soit combiné avec ledit manganèse et/ou avec ledit bismuth sous la forme de micro inclusions de MnTe et/ou Bi_{Z}Te₃ (excepté que lorsque le plomb est présent une partie du tellure peut être combinée avec le plomb sous la forme de micro inclusions de PbTe en des quantités insuffisants pour produire une fissuration sensible de la surface pendant le formage à chaud de ladite billette) et que ledit bismuth soit également présent sous la forme de micro inclusions de bismuth élémentaire, FeTe n'étant sensiblement pas présent dans ladite forme solide;
chauffer ladite forme en acier allongée à une température de déformation à chaud, sans brûler la forme en acier;
et déformer à chaud ladite forme allongée pendant que cette dernière est à une température au-dessus d'environ 920°C (1700°F) et au-dessous de 1150°C (2100°F).

2. Procédé selon la revendication 1 dans lequel ladite étape de coulée consiste à couler ledit acier fondu sous la forme d'un lingot; et ladite étape de déformation à chaud consiste à réchauffer ledit lingot et ensuite à laminer à chaud ledit lingot réchauffé en un méplat avec ledit lingot à une température de laminage à chaud au-dessus de 920°C (1700°F) et au-dessous de 1150°C (2100°F); aucune étape d'enlèvement de la surface n'existant entre ladite étape de réchauffage et ladite étape de laminage à chaud.

3. Procédé selon la revendication 2, et consistant en outre à réchauffer ledit méplat et ensuite à laminer à chaud ledit méplat à une température au-dessus de 920°C (1700°F) et au-dessous de 1150°C (2100°F) pour produire un méplat ayant une surface sensiblement exempt de fissuration de surface préalablement à tout traitement de surface de ce!ui-ci; aucune étape d'enlèvement de la surface n'existant entre ladite étape de réchauffage du méplat et ladite étape de laminage à chaud exposés en dernier.

4. Procédé selon la revendication 1 dans lequel ladite étape de coulée consiste à couler en continu ledit acier fondu sous la forme d'une bande; et ladite étape de déformation à chaud consiste à dégauchir par rouleaux ladite bande tandis que cette dernière est à une température au-dessus de 920°C (1700°F) et au dessous de 1100°C (2000°F).

5. Procédé selon l'une quelconque des revendications précédentes dans lequel ladite étape de déformation à chaud est réalisée à une température au-dessous de 1035°C (1900°F).

6. Procédé selon l'une quelconque des revendications précédentes dans lequel ledit acier contient en outre jusqu'à 0,15% en poids de plomb, et ladite teneur en tellure est de 0,02% en poids maximum, ledit acier dans ladite forme solide ayant des micro inclusions de PbTe en des quantités insuffisantes pour produire une fissuration sensible de la surface pendant ladite étape de déformation à chaud.

7. Procédé selon l'une quelconque des revendications précédentes dans lequel, lorsque le plomb est présent, la teneur en plomb plus bismuth combinée, est au moins de 0,25% en poids.

8. Billette telle que déformée d'acier exempt d'usinage caractérisé en ce que ladite billette comprend:
une composition comprenant en poids %:
tout ledit tellure étant combiné avec ledit manganèse et/ou avec ledit bismuth sous la forme de micro inclusions de MnTe et/ou de Bi₂Teₐ (excepté que lorsque le plomb est présent une partie du tellure peut être combinée avec le plomb sous la forme de micro inclusions de PbTe en quantités insuffisantes pour produire une fissuration sensible de la surface pendant le formage à chaud de ladite billette).
Il n'existe pratiquement pas de FeTe,
des micro inclusions de bismuth élémentaire;
une surface de billette pratiquement exemple de fissuration et de brûlure de la surface dans la condition telle que déformée;
et de l'oxyde de fer sur la surface de ladite billette dans ladite condition telle que déformée.

9. Billette selon la revendication 8 dans laquelle ledit acier contient jusqu'à 0,15% en poids de plomb, ladite teneur en tellure est 0,02% en poids maximum, ladite billette ayant des micro inclusions de PbTe en des quantités insuffisantes pour produire une fissuration de surface substantielle pendant la formation à chaud de ladite billette.

10. Billette selon la revendication 8 ou la revendication 9, dans laquelle lorsque le plomb est présent, la teneur en plomb plus bismuth combinés est au moins de 0,25% en poids.

11. Billette selon l'une quelconque des revendications 8 à 10 dans laquelle la quantité de micro inclusions de MnTe est suffisante pour causer la fissuration de surface pendant la déformation à chaud à des températures dépassant substantiellement 1 035°C (1900°F).

## Patentansprüche

1. Verfahren zum Herstellen eines langgestreckten, vorgearbeiteten tellurhaltigen Stahlformteils, der aufgrund von Bleitellurid vor Oberflächenbehandlung Oberflächenriß-frei ist, dadurch gekennzeichnet, daß das Verfahren die Schritte aufweist:
Bereitstellen eines Bades geschmolzenen Stahls mit einer Zusammensetzung (in Gew.-%):
Gießen des geschmozenen Stahls in eine längliche feste Form;
wobei der Stahl mit hinreichend Mangan und Wismuth versehen ist, so daß im festen Formteil das gesamte Tellur mit dem Mangan und/oder dem Wismuth als Miroeinschlüsse von MnTe und/oder Bi₂Teₐ (außer dann, wenn Blei anwesend ist, kann etwas Tellur mit Blei als Miroeinschlüsse von PbTe, in Mengen, die nicht hinreichend sind, um wesentliche Oberflächenrisse während des Heißformens des Stranges zu bewirken, verbunden sein) vorliegt, daß Wismuth auch als Mikroeinschlüsse elementaren Wismuths vorliegt, wobei in dem festen Formteil im wesentlichen kein FeTe anwesend ist;
Erhitzen des länglichen Stahlformteils auf eine Heißformtemperatur, ohne das Strahlformteil zu verbrennen; und
Heißverformen des länglichen Formteils, während sich letzteres bei einer Temperatur oberhalb etwa 920°C (1700°F) und unterhalb 1150°C (2100°F) befindet.

2. Verfahren, wie in Anspruch 1 beschrieben, wobei der Guß-Schritt das Gießen des geschmolzenen Stahls in einem Barren; und der Heiß-Verformungsschritt Wiederaufheizen des Barrens und anschließendes Heißwalzen des wiederaufgeheizten Barrens zu einem Strang, wobei sich der Barren bei einer Heißwalztemperatur oberhalb 920°C (1700°F) und unterhalb 1150°C (2100°F) befindet, wobei zwischen dem Wiederaufheizen und dem Heißwalzschritt kein Oberflächen-Entfernungsschritt vorliegt, aufweist.

3. Verfahren, wie in Anspruch 2 beschrieben, welches ferner das Wiederaufheizen des Walzblocks und anschließend Heißwalzen des Walzblocks bei einer Temperatur oberhalb von 920°C (1700°F) und unterhalb 1150°C (2100°F) aufweist, um einen Strang mit im wesentlichen oberflächenrißfreier Oberfläche herzustellen, bevor irgendeine Oberflächenbehandlung durchgeführt wird, wobei kein Oberfiächener<tfernungsschritt zwischen dem Schicht-Wiederaufheizschritt und dem zuletzt angegebenen Heiß-Walzschritt liegt.

4. Verfahren, wie in Anspruch 1 beschrieben, wobei der Gußschritt kontinuierliches StrangGießen des geschmolzenen Stahls; und der Heißverformungsschritt Walz-Begradigung des Stranges aufweist, während letzterer sich bei einer Temperatur oberhalb von 920°C (1700°F) und unterhalb von 1100°C (2000°F) befindet.

5. Verfahren, wie in einem der vorangehenden Ansprüche beschrieben, wobei der Heißverformungsschriftt bei einer Temperatur unterhalb 1035°C (1900°F) durchgeführt wird.

6. Verfahren, wie in einem der vorangehenden Ansprüche beschrieben, wobei der Stahl ferner bis zu 0,15 Gew.-% Blei aufweist und der Tellurgehalt maximal 0,02 Gew.-% beträgt, wobei der Stahl in fester Form Miroeinschlüsse von PbTe in Mengen besitzt, die nicht hinreichend sind, um wesentliche Oberflächenrißbildung während des Heißverformschrittes zu bewirken.

7. Verfahren, wie in einem der vorangehenden Ansprüche beschrieben, wobei dann, wenn Blei anwesend ist, der Gesamtgehalt Blei plus Wismuth mindestens 0,25 Gew.-% beträgt.

8. Derart geformter Automatenstahlstrang, dadurch gekennzeichnet, daß der Strang aufweist:
Eine Zusammensetzung, die in Gew.-% aufweist:
wobei das gesamte Blei mit dem Mangan und/oder dem Wismuth als Mikroeinschlüsse von MnTe und/oder Bi_{Z}Te₃ vorliegt (außer dann, wenn Blei anwesend ist, wobei etwas Tellur mit Blei als Mikroeinschlüsse von PbTe in Mengen anwesend sein kann, die nicht hinreichend sind, um wesentliche Oberflächenrißbildung während Heißformens des Barrens zu bilden); wobei im wesentlichen kein FeTe anwesent ist; elementares Wismuth in Form von Mikroeinschlüssen vorliegt; die Strangoberfläche im wesentlichen oberflächenrißfrei und verbrennungsfrei in geformtem Zustand vorliegt; und kein Eisenoxid auf der Oberfläche des Barrens im geformten Zustand anwesend ist.

9. Strang, wie in Anspruch 8 beansprucht, wobei der Stahl ferner bis zu 0,15 Gew.-% Blei enthält, der Teillurgehalt maximal 0,02 Gew.-% beträgt, und der Barren Mikroeinschlüsse von PbTe in unzureichenden Menge, um beträchtliche Oberflächenrißbildung während der Heißverformung des Barrens hervorzurufen, besitzt.

10. Strang, wie in Anspruch 8 oder 9 beschrieben, wobei dann, wenn Blei anwesend ist, der Bleiplus Wismuth-Gesamtgehalt mindestens 0,25 Gew.-% beträgt.

11. Strang, wie in einem der Ansprüche 8 bis 10 beschrieben, wobei die Menge MnTe-Mikroeinschlüsse hinreichend ist, um Oberflächenrißbildung während Heißverformung bei Temperaturen, die 1035°C (1900°F) wesentlichen überschreiten, zu bewirken.
